

## UNITED STATES PATENT OFFICE.

ANTON LEDERER, OF VIENNA, AUSTRIA-HUNGARY, ASSIGNOR TO WESTINGHOUSE LAMP COMPANY, A CORPORATION OF PENNSYLVANIA.

MANUFACTURE OF TUNGSTEN FILAMENTS FOR INCANDESCENT ELECTRIC LAMPS.

1,034,018.

Specification of Letters Patent. Patented July 30, 1912.

No Drawing.

Application filed June 8, 1909. Serial No. 500,955.

To all whom it may concern:

Be it known that I, ANTON LEDERER, a subject of the Emperor of Austria-Hungary, and a resident of Vienna, Austria-Hungary, have invented a new and useful Improvement in the Manufacture of Tungsten Filaments for Incandescent Electric Lamps, of which the following is a specification.

In the specification of my application for 10 Letters Patent, Serial No. 313,485, I have described a process for the manufacture of pure tungsten filaments which consists in making a plastic mass from tungsten dioxid, and a suitable binding material, such as an 15 ammoniacal solution of casein, a solution of isinglass, levulose, etc., in such proportions that the whole of the carbon of the binding material may be removed by the oxygen of the tungsten dioxid. From this mass filaments are squirted which are then heated in 20 the absence of oxidizing gases, so that the carbon is removed and pure tungsten filaments obtained. I have found from experience that such filaments only become sufficiently strong for further manipulation 25 when the heating is conducted at a temperature considerably in excess of the temperature necessary for reduction.

The object of the present invention is to 30 obviate heating the filaments at this stage to an excessive temperature, and I have found that by adding powdered metallic tungsten to the paste of tungsten dioxid and binding material, the filament is sufficiently strong 35 for the later manipulations without it being necessary to heat to a temperature exceeding that at which the reduction takes place.

In accordance with my invention a suitable quantity of powdered tungsten metal 40 is added to the paste consisting of tungsten dioxid and carbonaceous binding material. This paste is then squirted through dies and the filaments obtained are heated to the temperature necessary for the reduction of 45 the tungsten dioxid. This temperature is amply sufficient to give the filaments the strength necessary for the further manipulation. The addition of tungsten metal to the paste does not in any way influence the 50 action described in my previous specification above mentioned by means of which the carbon is removed because only the carbon of the binding agent and the oxygen of the tungsten dioxid take part in the reaction.

This reaction may be conveniently expressed 55 by the following equation:



Since the agglutinants mentioned in the opening paragraph of the specification possess great binding qualities, the process herein described can be easily carried out. although a smaller proportion of agglutinant is employed. I have in fact discovered that in certain circumstances particularly when 60 manufacturing filaments of large cross section, which sinter together less easily, it is advantageous to take a smaller quantity of binding agent than is necessary for the complete reduction of the tungsten dioxid used, 70 and in order to effect a complete reduction of the oxid it is then necessary to make up the deficiency by adding to the mixture a sufficient quantity of pure carbon, for instance graphite, lamp-black or soot. It is 75 of course obvious that in such cases care must be taken when making an addition of pure carbon to have a sufficient quantity of tungsten dioxid in the paste to supply the necessary amount of oxygen to oxidize all the 80 carbon. The filaments thus obtained are then heated to incandescence in a suitable environment by passage through them of an electric current for the purpose of completing the reduction of any oxid they may still 85 contain and for sintering them.

I claim as my invention:

1. The process of manufacturing homogeneous tungsten filaments for incandescent electric lamps which consists in preparing 90 a paste of tungsten dioxid and a suitable carbonaceous binding material in such proportions that the carbon of the binding material is approximately sufficient to combine with the oxygen of the tungsten dioxid, incorporating powdered tungsten metal with the paste for the purpose of facilitating the reduction of the tungsten dioxid by the carbon of the binding material, squirting said paste into filaments, drying the same, heating said filaments in the absence of oxidizing gases to the temperature necessary for reduction and thereafter finishing the metal filaments produced in a suitable manner, substantially as described.

2. The process of manufacturing homogeneous tungsten filaments for incandescent electric lamps which consists in preparing a

paste of tungsten dioxid and a suitable carbonaceous binding material in such proportions that the carbon of the binding material is approximately sufficient to combine 5 with the oxygen of the tungsten dioxid, incorporating powdered tungsten metal with the paste for the purpose of facilitating the reduction of the tungsten dioxid by the carbon of the binding material, squirting said 10 paste into filaments, drying the same, heating said filaments in the absence of oxidizing gases to the temperature necessary for reduction and heating said filaments to incandescence by passage therethrough of an 15 electric current in a suitable environment, substantially as described.

3. The process of manufacturing homogeneous tungsten filaments for incandescent electric lamps which consists in preparing a 20 paste of tungsten dioxid and a suitable carbonaceous binding material and carbon in

such proportions that the total carbon is approximately sufficient to combine with the oxygen of the tungsten dioxid, incorporating powdered tungsten metal with the paste 25 for the purpose of facilitating the reduction of the tungsten dioxid by the carbon of the binding material, squirting said paste into filaments, drying the same, heating said filaments in the absence of oxidizing gases to 30 the temperature necessary for reduction and heating said filaments to incandescence by passage therethrough of an electric current in a suitable environment, substantially as described. 35

In testimony whereof I have hereunto subscribed my name this 3rd day of June 1909.

ANTON LEDERER.

Witnesses:

CHARLES A. TERRY,  
Wm. H. CAPEL.